

Dec. 4, 1928.

1,694,189

S. RUBEN

PHOTOSENSITIVE CELL

Filed Dec. 6, 1927

*Fig. 1.*



*Fig. 2.*



Inventor  
SAMUEL RUBEN

By his Attorney *M. W. Clephane*

## UNITED STATES PATENT OFFICE.

SAMUEL RUBEN, OF NEW YORK, N. Y.

## PHOTORESITIVE CELL.

Application filed December 6, 1927. Serial No. 238,217.

This invention relates to a photo-sensitive cell and to the method of making the photo-sensitive element thereof.

The object of the invention is the provision 5 of an accurately responsive and durable cell of this type.

It is known that cuprous oxide, when formed in a particular way is photo-electrically sensitive; it is also known that because of its high specific resistance when so employed it must be used in a thin layer on 10 a supporting base.

Broadly, my invention consists of a tube evacuated to a pressure at which substantially 15 no positive ionization occurs, and having three electrodes, cathode, anode and grid, the last of which comprises a copper body having on its surface a fused layer of cuprous oxide which is made in the manner herein- 20 after described, and which is electrically highly sensitive to light rays. In this device the grid is operated through the intermittent exposure of the cuprous oxide surface to light rays thereby varying its electrical resistance 25 and correspondingly, its potential, employed to vary the distribution of the electron stream over the plate surface, and therefore the current flow in the cathode-anode circuit.

I have found that for most effective photo- 30 electric application the cuprous oxide layer on the copper base must have minimum specific resistance and maximum crystal layer density, to obtain which, by the method of my invention, a copper body is heated in an oxidizing atmosphere to 1000° C., and when a fused cuprous oxide coating of about 0.1 mm. has thus been formed on the base surface, it is plunged into a 25% solution of hydrochloric acid, when it forms a dense, clear, 40 red, glass-like, cuprous oxide coating which is firmly adherent to the base. It is obvious that any undesirable reaction product remaining on the surface after the quenching of the hydrochloric acid should be entirely removed 45 either mechanically or chemically in order to present the cleanest red cuprous oxide surface possible. This layer is chemically pure and has a relatively low specific resistance compared with that of such a compound prepared by the methods now known, as for example, by heating the copper to a high temperature and allowing it to slowly cool in the air, when there is formed a layer of cupric oxide outside of the cuprous oxide coating. 50

The outer layer has a higher resistance than

the cuprous oxide and is not satisfactory for photoelectric use.

Because of the polarized character of the cuprous oxide layer formed, and especially when quenched by the method of my invention, excellent asymmetrical conductivity is shown in a cell using this material as a separating element. This factor is to be taken into account in the electrical connection and use of the element in a photoelectric cell. 60 65

In view of the very thin layer employed and of the necessity for exposing the maximum amount of surface to the radiations to be indicated, it is preferable to use this layer in the form described, as in a vacuum tube, 70 to control the flow of ionic or electronic discharge. Below I describe a preferred form of photoelectric cell utilizing the photoelectric cuprous oxide layer to control an electric discharge by resistance variations of its 75 surface layer responsive to exposure to light rays. To minimize the effect of possible radiations from a source of electron emission in a device of this character, there is employed a filament or electron emission cathode having as its electron emission surface a layer 80 of alkaline earth oxides, such as strontium and barium oxides which allows a cathode operation at a low temperature or at a dull red heat. In this respect the combination of a 85 photo-sensitive resistance element and a low temperature cathode is equivalent to that cited in my prior and copending application, bearing Serial Number 534,213.

In the accompanying drawings, illustrative 90 of one embodiment of the invention, Fig. 1 shows in outline a vacuum tube equipped with a photo-sensitive electrode and other electrodes, connected in an electric circuit and Fig. 2 is a section view of the electrode at 95 2-2.

At 1 is a filamentary cathode coated with strontium and barium oxides and supported by leads 1<sub>1</sub> and 1<sub>2</sub>, and mounted on lead 2, edgewise to the cathode is anode 2, and extending upon two sides of and parallel with the anode is the grid or control element 3, composed of a copper strip having fused on its surface a coating of light sensitive cuprous oxide. At B is the source of heat energy for the cathode, and B<sub>1</sub> is the source of potential between the cathode and grid, B<sub>2</sub> being the source of potential between the cathode and anode and R the resistance in that circuit. 100 105

In operation, as light is impressed upon 110

the grid element, causing changes in its initial resistance, corresponding changes occur in the potential in the grid circuit, in this way controlling the electron stream bombarding the anode. Thus, the cathode-anode current discharge is varied in response to changes in the external light rays impinging upon the cuprous oxid grid coating.

What I claim is—

- 10 1. In a photoelectric cell, the combination of a cathode, an anode and a control electrode composed of a copper body having a surface of fused cuprous oxide.
- 15 2. The method of making a photo-sensitive electrode which consists in heating a copper body to 1000° C. while exposed to the air and quenching it in a 25 per cent solution of hydrochloric acid.
- 20 3. The method of producing a photo-sensitive resistance element which consists in heating a copper body until a fused layer of cuprous oxide is formed on its surface, and quenching it in a solution of hydrochloric acid.
- 25 4. The method of producing a photo-sensitive electrode which consists in heating a copper body in an oxidizing atmosphere until there is a layer on said body of an integrally formed homogeneous non-porous crys-

talline compound of said copper body, and 30 quenching it.

5. In a photo electric cell, a cathode, an anode and a control electrode consisting of cuprous oxide.

6. In a photo electric cell, a cathode, an 35 anode and a control electrode consisting of fused cuprous oxide.

7. In a photo electric cell, a cathode, an 40 anode and a control electrode consisting of a metal base having an exposed surface of substantially cuprous oxide.

8. In a photo-electric cell, a resistance control electrode consisting of a metal base having an exposed surface of fused cuprous oxide.

9. In an electron discharge device, an element for controlling the impedance of said device, having a surface of integrally formed, 45 homogeneous, non-porous crystalline cuprous oxide.

10. In an electrical discharge tube, a cathode, an anode and a control element consisting of cuprous oxide.

In testimony whereof, SAMUEL RUBEN has signed his name to this specification this 5th 50 day of December, 1927.

SAMUEL RUBEN.